

United States Patent [19]  
Jones

[11] 3,900,316  
[45] Aug. 19, 1975

[54] CASTABLE NICKEL-CHROMIUM  
STAINLESS STEEL

[75] Inventor: Robin Mackay Forbes Jones,  
Suffern, N.Y.

[73] Assignee: The International Nickel Company,  
Inc., New York, N.Y.

[22] Filed: Mar. 7, 1973

[21] Appl. No.: 337,278

**Related U.S. Application Data**

[63] Continuation-in-part of Ser. No. 275,095, Aug. 1,  
1972, abandoned, which is a continuation-in-part of  
Ser. No. 182,219, Sept. 20, 1971, abandoned.

[52] U.S. Cl. .... 75/128 A; 75/125; 75/128 C;  
75/128 F; 75/128 G; 75/128 P; 75/128 W

[51] Int. Cl.<sup>2</sup> .... C22C 38/02; C22C 38/08;  
C22C 38/54; C22C 38/58

[58] **Field of Search** .... 75/128 A, 128 C, 128 F,  
75/125, 128 G, 128 P, 128 W; 148/38

[56] **References Cited**

UNITED STATES PATENTS

2,432,616 12/1947 Franko .... 75/128 F

|           |         |                     |          |
|-----------|---------|---------------------|----------|
| 2,590,835 | 4/1952  | Kirkby .....        | 75/128 F |
| 2,743,175 | 4/1956  | Talbot .....        | 75/128 F |
| 2,879,194 | 3/1959  | Eischelberger ..... | 75/128 F |
| 3,112,195 | 11/1963 | Souresny .....      | 75/128 F |
| 3,199,978 | 8/1965  | Brown et al. ....   | 148/38 X |
| 3,352,666 | 11/1967 | Foster .....        | 75/125   |
| 3,552,950 | 1/1971  | Rundell.....        | 75/125   |
| 3,754,899 | 8/1973  | Kanter .....        | 75/128 F |
| 3,806,337 | 4/1974  | Jones .....         | 75/128 A |

*Primary Examiner*—L. Dewayne Rutledge

*Assistant Examiner*—Arthur J. Steiner

*Attorney, Agent, or Firm*—George N. Ziegler; Ewan C. MacQueen; Raymond J. Kenny

[57]

**ABSTRACT**

Nickel-chromium stainless steel containing, inter alia, nickel, chromium, silicon and boron in specially correlated proportions is characterized by particularly good castability along with strength and corrosion resistance for production of strong corrosion-resistant castings in sand or metal molds.

**16 Claims, No Drawings**

## CASTABLE NICKEL-CHROMIUM STAINLESS STEEL

This application is a continuation-in-part of U.S. Application Ser. No. 275,095, filed Aug. 1, 1972, which is a continuation-in-part of U.S. Application Ser. No. 182,219, filed Sept. 20, 1971, both of which are abandoned.

The present invention relates to nickel-chromium-stainless steels and more particularly to austenitic nickel-chromium stainless steels for castings.

As is known it is often desirable to produce austenitic nickel-chromium steels by casting methods, particularly where the desired article is of a complex shape that is difficult or expensive to forge or machine. Usually, stainless steels are cast in sand molds or other expendable refractory molds, e.g., investment molds or resin-bonded shell molds, inasmuch as the castability characteristics of these steels generally require pouring at temperatures at least as high as about 2,750°F. and usually higher, e.g., 2,950°F. or 3,100°F., especially when the casting has relatively long thin sections of one-fourth inch or one-eighth inch or less in thickness.

While many varieties of stainless steels have been successfully cast, it has been evident that much better castability, particularly for producing thin-sectioned stainless steel castings, would be very beneficial. Furthermore, inasmuch as stainless steels have characteristics that are frequently desired in castings which are needed in large quantities it has been, and still is, highly desirable to have an austenitic nickel-chromium stainless steel that could be cast by permanent mold casting or die casting in cast iron or steel, or even molybdenum or graphite, molds in order to obtain economic advantages from repeated use of a mold and also in order to achieve dimensional accuracies obtainable with metal molds. Economic advantages of permanent mold casting and die casting are contingent upon repeated utilization of "permanent" casting cavity to produce castings having high quality surfaces.

However, if the permanent mold or die becomes heat crazed, the surface quality of the castings is poor. A major factor which influences heat crazing of dies is the pouring temperature of the casting alloy. And, in order to obtain good castings throughout repeated use of a mold over a long period of life, and also in order to amortize the cost of the mold over a large number of castings, it is especially desirable to have an alloy that can be cast in thin sections at temperatures not greatly above the melting temperatures of commercial die steels. It is particularly desirable to have good castability at pouring temperatures of about 2,650°F. or lower, this being in marked contrast to the significantly conventional temperature of 2,750°F. to 3,100°F. noted above. Good castability includes the capability of molten metal to run through thin sections of a mold and, very importantly, also to flow and merge cleanly into itself when the flow of metal in the mold divides and then merges together, in which circumstance it is especially important to obtain complete sound solidification without colds shuts, folds or oxide films. Also, cleanliness in the molten condition and a low melting point are desirable characteristics for good castability.

But to achieve the foregoing should not be at the cost of losing necessary mechanical properties and corrosion resistance. For general use in industry, building construction and household use and for many other

purposes it is desirable that a cast stainless steel have at least modest mechanical strength and ductility characteristics, e.g., 60,000 psi ultimate tensile strength, 25,000 psi yield strength with about 5% or more tensile elongation. It is also desirable that a steel casting have impact resistance to withstand rough handling such as by being dropped on a concrete floor or hammered to conform it in an assembly. Although this does not necessitate 5% elongation, the cast steel should be characterized by at least 1% elongation in order to satisfy minimal requirements, such as decorative and other nonstructural uses. Good general corrosion resistance includes resistance to staining in corrosive atmosphere, e.g., salt spray. Moreover, for industrial production of castings, especially highly intricate castings or castings made in metal molds, it is important that a steel not suffer from excessive hot shortness.

There has now been discovered a nickel chromium stainless steel which has good characteristics for producing strong corrosion-resistant castings at desirably low pouring temperatures.

It is an object of the present invention to provide a nickel-chromium stainless steel casting.

A further object of the invention is to provide a process for producing strong corrosion-resistant stainless steel articles.

Other objects and advantages will become apparent from the following description.

The present invention contemplates nickel-chromium stainless steel castings, and also alloys and processes for production thereof, containing by weight, about 6% to 30% nickel, about 14% to about 26% chromium, up to about 0.15% carbon, advantageously not more than 0.1% carbon, about 2% to 5% silicon, advantageously 2.8% to 3.8% silicon, up to about 20% manganese, at least 0.2% boron, e.g., about 0.25% or 0.3%, to about 1.4% boron, up to about 3% copper, up to about 8% molybdenum, up to about 1.4% phosphorus and up to about 1% columbium and wherein the amounts of nickel, manganese, chromium, molybdenum, silicon, boron and phosphorus in this subject composition are correlated according to the relationship

$$8(\%Ni+\%Mn)-1.5(\%Cr+Mo)+22(-\%Si)+284(\%B)+189(\%P) \text{ equal at least } 360. R(1)$$

Excellent castability characteristics that are beneficial for the melting and pouring of castings are obtainable with the subject alloy composition. Embodiments of the subject alloy have been successfully melted in gas-fired furnaces and cast at 2,350°F. in green sand molds and good filling, with sharp definition at corners, was achieved in thin-sectioned mold cavities about three-sixteen inch thick by 1½ inches square. To achieve excellent castability the composition is advantageously correlated to provide that the foregoing relationship R(1) equals at least 560.

For certain other advantages, such as especially good ductility or corrosion resistance or low cost along with good (although not maximum) fluidity, the invention provides a restricted range composition containing about 6% to 26% or 28% nickel, about 14% to 20% or 25% chromium, up to about 0.15% carbon, advantageously not more than 0.1% carbon, about 2% to 5% silicon, advantageously 2.8% to 3.8% silicon, up to about 20% manganese, 0.3% to about 0.7% boron, up

to about 3% copper, up to about 8% molybdenum and up to about 1% columbium and wherein the amounts of nickel, manganese, chromium, molybdenum, silicon and boron are correlated in accordance with the relationship

$$8(\%Ni+\%Mn)-1.5(\%Cr+\%Mo)+22(\%Si)+284(\%B) \text{ equal at least 360.} \quad R(2)$$

Phosphorus in amounts up to 1.4% can be added to the restricted composition; when the alloy contains a substantial amount of phosphorus, e.g., 0.2%, 0.5% or more, a phosphorus term "+189(%P)" may be included in R(2).

Further, it is specially beneficial for obtaining desirable ductility characteristics, e.g., tensile elongation of at least 5% in the rapidly solidified and solution treated condition, to have the composition controlled according to the restricted range and R(2) and also correlated in accordance with the relationship

$$0.9(\%Si)+3.4(\%Cr)+(\%Mn)[33-(\%Mn)] \text{ equal or is less than 360.} \quad R(3)$$

While the balance of the steel is hereinafter referred to as iron, or essentially iron, it is to be understood the balance usually includes small amounts of impurities and incidental elements, including residuals of melt treating agents. Thus, the balance may include, for instance, up to 0.04% phosphorus, up to 0.04% sulfur, and up to 0.25% selenium. Nitrogen may be present in amounts up to the solubility limit, e.g., up to about 0.25% nitrogen. Such highly oxidizable elements as titanium and aluminum are desirably avoided or carefully limited to low levels, e.g., 0.3% or less, in the steel of the present invention inasmuch as substantially greater amounts of these elements, either as metals or oxides, would be detrimental to the good castability characteristics of the steel. In this regard, it is of advantage that the present steel provides satisfactory sound castings, free from porosity and with good strength and ductility, without need for titanium. Small additions of aluminum, e.g., 0.1% aluminum, are effective for deoxidation. However, substantially greater amounts of aluminum would adversely affect castability and, accordingly, large additions or progressive build-up of aluminum are avoided and the amount of aluminum in the steel should not exceed about 0.3%. For good castability characteristics it is beneficial to maintain the steel essentially devoid of titanium, or with not more than 0.1% titanium, and to restrict the total amount of any aluminum and titanium to not greater than 0.2%.

Small additions of selenium, e.g., 0.015% to 0.03%, when finishing melts of the steel are recommended for obtaining sound castings, especially for avoiding pin-hole porosity in green sand castings. Frequently very little of the selenium remains in the steel, e.g., residual selenium of less than 0.01% in a casting from a melt which had an effective addition of 0.02% selenium.

The steel of the invention is especially characterized by very good or excellent castability enabling production of complex thin-sectioned stainless steel castings with the steel poured, or cast, at temperatures of about 2,650°F. or 2,350°F. or lower. Among the good castability characteristics, it is particularly notable that the steel is clean and essentially free from films, dross,

scum, etc. when held molten or cast in air at 2,650°F. or 2,350°F. or somewhat lower and knits or blends cleanly with itself in turbulent mold flow conditions. Also, the steel is fully molten at temperatures down to 2,350°F. or lower, such as 2,150°F. when the steel contains at least 0.8% each of boron and phosphorus and R(1) is at least 560. Thus, it is to be understood that, as a practical matter, the steel of the invention is characterized by a "freezing" temperature (incipient freezing or, approximately, the liquidus) not higher than 2,350°F. For example, the freezing temperature of a steel of the invention, namely alloy No. 8 which is referred to hereinafter in Tables I and II, was determined by thermocouple measurement to be 2,322°F.

The striking cleanliness characteristics are decidedly attractive for melting and casting in air using conventional induction furnaces or arc furnaces and foundry ladles. Vacuum melting may be used if desired for some purpose. Gas-fired melting was successful for steels of the invention containing more than 0.7% each of boron and phosphorus and with R(1) at least about 715. Castings of the subject steel can be poured in practically all kinds of expendable foundry molds, e.g., green sand molds, dry sand molds, resin-bonded shell and investment molds. But of special commercial significance is the advantage, e.g., as where close dimensional control and repeated use of molds is required, that the steel can be cast in permanent molds or die casting molds made of cast iron or steel, or of graphite or molybdenum. Testing of embodiments containing 0.3% to 0.7% boron has shown that these steels have good resistance to hot tearing and avoid hot-shortness. Good results, including smooth surface finish and complete sound solidification with very good filling of thin sections and fine details in the mold, have been obtained when casting the steel of the invention in green sand molds and also in permanent iron molds.

For production in sand foundries where gas-fired melting is not essential and good castability for making sand castings, rather than die castings, is of primary importance, the R(1) factor can be as low as 180. Furthermore, for benefiting surface finish, castability and ductility of sand castings, the manganese content is advantageously controlled to a range of 0.1 to 5.

A particularly good composition for economical production of sand casting contains about 8% to 14% nickel, 16% to 20% chromium, 2.5% to 3.5% silicon, 0.25% to 0.55% boron, up to 0.15% carbon, 0.2% to 2.5% manganese, up to about 4% molybdenum, up to 2% copper and balance iron and with the composition correlated in accordance with the relationship

$$8(\%Ni+\%Mn)-1.5(\%Cr+\%Mo)+22(-\%Si)+284(\%B)+189(\%P) \text{ equal at least 180.} \quad R(4)$$

The cast steel of the invention has satisfactory strength and ductility, e.g., room temperature yield strength of 25,000 or 30,000 psi or more at 0.2% offset, and also corrosion resistance, for many industrial or household or other commercial uses. With the restricted composition containing 0.3% to 0.7% boron and incidental amounts of phosphorus, a desirable room temperature ductility characteristic of at least 5% tensile elongation is obtainable with the steel cast in thin sections and solution treated, e.g., a 1/4 inch thick cross-section cast in a dry sand mold and solution treated 1 hr. at 2,000°F. Ductility characteristics are, in

general, benefited by rapid solidification from the molten condition such as when cast in thin sections and/or in metal molds and are also benefited by solution heat-treatment after solidification. A recommended range for solution treatment is 1,850°F. to 2,050°F. for one-half hour or longer, e.g., 1 hour, followed by air cooling, or more rapid cooling, down to 600°F. or lower, e.g., room temperature.

In the as-cast condition the microstructure of the steel is normally characterized by dendrites composed of austenite, ferrite, etc., with intermetallic precipitates, e.g., acicular borides and/or eutectic phosphides, in the interdendritic regions. The solution-treated condition of the cast steel is usually characterized by a dendritic microstructure comprising substantially less precipitate than in the cast condition. Grain sizes of the castings and also the sizes and distributions of the microstructure particles are generally smaller and finer, e.g., interdendritic spacing of about 10 to 50 microns, and more uniformly distributed, in the rapidly solidified castings. The solution-treated structure is advantageous for good ductility and corrosion-resistant characteristics of the steels with 0.3% to 0.7% boron.

In reference to the composition of the steel it is particularly noted that the steel contains at least 6% nickel, and more desirably at least about 8% nickel, to provide, where desired, a stable austenitic structure in practical conditions of use. Moreover, the nickel content also promotes desirable ductility characteristics, including shock resistance, and corrosion resistance of the castings. In these respects, at least about 8% nickel, more advantageously at least 11% nickel, in the steel is advantageous.

The silicon content does not exceed 5% in order to avoid adverse effects on ductility. For consistently achieving good ductility, silicon should be not greater than 3.8%. Compositions with silicon contents of 2.5% to 3.8% and boron contents of 0.3% to 0.7% are recommended for a particularly advantageous combination of castability and ductility characteristics.

The stainless steels include 0.3% to about 1.4% boron and about 14% to 25% chromium, advantageously at least 0.45% boron and at least 17.5% chromium, to contribute the combination of castability, ductility and corrosion resistance which characterize the composition as a whole. Embodiments containing 0.3% to 0.7% boron are desirable from the viewpoint of ductility and corrosion resistance; embodiments containing more than 0.7% boron, e.g., 0.8% boron, particularly 0.9% to 1.3% boron, are recommended from the fluidity viewpoint; and, where castability needs are dominant, embodiments containing a combination of 0.9% to 1.4% phosphorus along with 0.9% to 1.4% boron are advantageous for obtaining excellent castability and also for enabling melting in gas-fired foundry furnaces.

The steel usually contains at least about 1% manganese, often about 5% or 10% or more manganese, in order to benefit castability and ductility.

Small amounts of carbon, e.g., at least about 0.02%, are advantageous for enhancing the castability of the steel.

Presence of copper in the steel, e.g., about 1.5%, 2%, or 2.7% copper, is desirable for benefiting corrosion resistance, particularly resistance to sulfuric acid solutions. Molybdenum, e.g., about 2% to 6%, is desirably present for enhancing resistance of the steel to corrosive attack, particularly crevice corrosion and pitting

corrosion in chloride media. However, excessive amounts of copper and/or molybdenum, e.g., 4% copper, should be avoided in order to avoid embrittling the steel.

5 In carrying the invention into practice, an especially desirable combination of castability, strength, ductility and corrosion resistance, along with other beneficial characteristics, is obtained with a specially advantageous composition containing 8% to 10% nickel, 17.5% to 19.5% chromium, 0.02% to 0.1% carbon, 2.75% to 3.25% silicon, 16% to 18% manganese, 0.45% to 0.7% boron, 1.5% to 2.5% copper and balance essentially iron and wherein the composition is further controlled in accordance with the relationship

$$15 \quad 8(\%Ni + \%Mn) - 1.5(\%Cr + \%Mo) + 22(\%Si) + 284(\%B) \\ \text{equal at least 385.} \quad R(4)$$

Moreover, with this specially advantageous composition, the steel of the invention is generally characterized in the solution treated condition by at least 30,000 psi yield strength, about 5 ft. lb. or more impact strength, a freezing temperature not greater than 2,325°F. and particularly good resistance to corrosion in salt spray media.

20 25 The invention further provides another advantageous steel which contains 23.5% to 26% nickel, 18% to 20% chromium, 3% to 3.5% silicon, 1% to 2% manganese, 0.02% to 0.08% carbon, 0.55% to 0.7% boron, 2.2% to 2.7% copper and 2.3% to 6.5% molybdenum and is especially beneficial for achieving very good corrosion resistance, particularly resistance to staining in salt spray, along with room temperature ductility of at least 5% tensile elongation and highly beneficial castability characteristics including a castable molten condition at 30 35 temperatures below 2,300°F., e.g., freezing temperatures of 2,290°F., 2,250°F. or even down to 2200°F. or lower.

For the purpose of giving those skilled in the art a further understanding of the invention, the following illustrative examples are given.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9

yses of melts of cast steels (Alloys) produced in accordance with the invention are set forth in the following Tables I and IA.

ported to contain 0.051% carbon, 12.8% nickel, 19.7% chromium, 3.8% silicon, 1.17% manganese, 0.53% boron and 0.029% phosphorus.

TABLE I

| Alloy No. | Composition - Weight Percent |      |      |      |      |      |      |     |      |
|-----------|------------------------------|------|------|------|------|------|------|-----|------|
|           | C                            | Ni   | Cr   | Si   | Mn   | B    | Cu   | Mo  | Fe   |
| 1         | 0.070                        | 8.3  | 16.1 | 3.10 | 17.8 | 0.49 | 2.12 | NA  | Bal. |
| 2         | 0.073                        | 8.5  | 15.9 | 3.04 | 17.8 | 0.48 | 2.15 | NA  | Bal. |
| 3         | 0.08                         | 8.4  | 14.8 | 3.2  | 17.7 | 0.46 | 2.16 | NA  | Bal. |
| 4         | 0.072                        | 8.3  | 14.0 | 2.55 | 16.1 | 0.33 | 2.15 | NA  | Bal. |
| 5         | 0.065                        | 8.0  | 15.8 | 3.10 | 16.0 | 0.33 | 2.09 | NA  | Bal. |
| 6         | 0.063                        | 8.4  | 17.4 | 4.10 | 15.8 | 0.38 | 2.16 | NA  | Bal. |
| 7         | 0.064                        | 8.3  | 15.9 | 2.5  | 17.4 | 0.39 | 2.08 | NA  | Bal. |
| 8         | 0.065                        | 8.6  | 16.8 | 3.35 | 17.5 | 0.39 | 2.14 | NA  | Bal. |
| 9         | 0.066                        | 8.4  | 14.2 | 4.10 | 17.6 | 0.36 | 2.07 | NA  | Bal. |
| 10        | 0.067                        | 8.3  | 16.8 | 2.45 | 19.7 | 0.34 | 2.02 | NA  | Bal. |
| 11        | 0.071                        | 8.3  | 14.3 | 3.29 | 19.1 | 0.37 | 2.12 | NA  | Bal. |
| 12        | 0.072                        | 8.5  | 14.6 | 4.25 | 19.9 | 0.39 | 2.13 | NA  | Bal. |
| 13        | 0.096                        | 8.3  | 15.2 | 3.05 | 16.9 | 0.45 | 2.11 | NA  | Bal. |
| 14        | 0.067                        | 25.3 | 18.8 | 3.0  | 1.9  | 0.57 | 2.38 | 2.3 | Bal. |
| 15        | 0.070                        | 25.7 | 18.7 | 3.1  | 1.8  | 0.63 | 2.58 | 4.5 | Bal. |
| 16        | 0.072                        | 23.5 | 18.7 | 3.2  | 1.8  | 0.68 | 2.46 | 6.5 | Bal. |
| 17        | 0.069                        | 14.5 | 18.8 | 3.2  | 5.9  | 0.58 | 2.25 | 2.3 | Bal. |
| 18        | 0.076                        | 11.4 | 18.8 | 3.2  | 10.1 | 0.61 | 1.86 | 2.3 | Bal. |
| 19        | 0.079                        | 9.8  | 18.7 | 3.2  | 16.0 | 0.68 | 2.16 | 2.3 | Bal. |
| 20        | 0.082                        | 8.8  | 15.0 | 3.04 | 18.3 | 0.47 | 2.21 | NA  | Bal. |

N.A. = Not Added and Not Analyzed

Bal. = Balance with impurities and residuals, including small amounts of up to 0.08% aluminum, 0.01% phosphorus, 0.015% sulfur and trace amounts of selenium not greater than 0.01%.

TABLE IA

| Alloy No. | Composition - Weight Percent |      |      |      |      |      |      |    |      |      |
|-----------|------------------------------|------|------|------|------|------|------|----|------|------|
|           | C                            | Ni   | Cr   | Si   | Mn   | B    | Cu   | Mo | P    | Fe   |
| 21        | 0.080                        | 8.5  | 15.7 | 3.30 | 18.5 | 0.89 | 2.11 | NA | 0.94 | Bal. |
| 22        | 0.091                        | 18.1 | 15.7 | 3.01 | 10.4 | 1.1  | 1.47 | NA | 1.1  | Bal. |
| 23        | 0.088                        | 17.0 | 15.6 | 3.06 | 10.4 | 1.1  | 1.48 | NA | 1.1  | Bal. |
| 24        | 0.087                        | 25.0 | 15.6 | 2.87 | 2.4  | 1.1  | 1.50 | NA | 1.1  | Bal. |
| 25        | 0.085                        | 25.0 | 15.5 | 2.91 | 2.3  | 1.1  | 1.52 | NA | 1.2  | Bal. |
| 26        | 0.089                        | 25.0 | 25.3 | 3.09 | 2.4  | 1.3  | 1.58 | NA | 1.3  | Bal. |
| 27        | 0.084                        | 25.6 | 25.6 | 2.96 | 2.3  | 1.3  | 1.57 | NA | 1.3  | Bal. |

N.A. = Not Added and Not Analyzed

Bal. = Balance with impurities and residuals, including small amounts of up to 0.08% aluminum, 0.015% sulfur and trace amounts of selenium not greater than 0.01%.

Further, four melts (alloys 28 to 31) were made with nominal compositions having a balance of iron and each with 0.08% carbon, 1% manganese, 18.5% chromium and 0.025% phosphorus and with other elements as follows: alloy 28 - 10.5% nickel, 2% silicon, 0.5% boron; alloy 29 - 10.5% nickel, 2% silicon, 0.3% boron; alloy 30 - 12% nickel, 3% silicon, 0.5% boron; and alloy 31 - 12% nickel, 3% silicon, 0.3% boron. Chemical analyses reported for the boron contents of alloys 28, 29, 30 and 31 were 0.48%, 0.25%, 0.51%, and 0.28% boron, respectively.

Another melt, alloy 32, was made by melting stainless steel scrap and adding alloying elements to prepare alloy 32 of the invention which, when analyzed, was re-

Results of room temperature tensile, impact and/or hardness testing of specimens machined from castings made of alloys in accordance with the invention (embodiments) are set forth in the following Table II. Alloys 4 to 12, 28 to 31 were cast in both 1-inch and  $\frac{1}{4}$ -inch or  $\frac{3}{8}$ -inch width keel block molds (alloys 4 to 12 and one-fourth-inch and alloys 28 to 31 in three-eighth-inch), and others were cast in either the 1-inch or one-fourth-inch widths; then, one-half-inch diameter and/or one-eighth-inch diameter tensile test specimens (2-inch and 1-inch gage lengths respectively) machined therefrom were tested. The results, as set forth in Table II, show particularly satisfactory mechanical properties of rapidly solidified steels cast in thin cross-sections.

TABLE II

| Alloy No. | Condition (X-Sect.)    | YS (ksi) | UTS (ksi) | Elong. (%) | R.A. (%) | Impact (ft.-lbs.) |
|-----------|------------------------|----------|-----------|------------|----------|-------------------|
| 1         | A-C(1")                | 37.5     | 72.6      | 8.0        | 9.5      | 5.5               |
| 1         | S.T.(1")               | 33.6     | 77.3      | 17.5       | 16.5     | 9.0               |
| 3         | A-C(1")                | 37.8     | 74.6      | 13.5       | 14.0     | —                 |
| 3         | S.T.(1")               | 34.9     | 74.1      | 14.5       | 16.0     | —                 |
| 4         | A-C(1")                | 31.7     | 61.2      | 10.0       | 13.0     | 12.5              |
| 4         | S.T.(1")               | 30.1     | 69.4      | 17.0       | 18.5     | 21.0              |
| 4         | A-C( $\frac{1}{4}$ ")  | 37.1     | 82.3      | 27.5       | 31.5     | —                 |
| 4         | S.T.( $\frac{1}{4}$ ") | 33.9     | 87.5      | 42.0       | 45.5     | —                 |
| 5         | A-C(1")                | 35.6     | 80.0      | 18.5       | 17.5     | 7.0               |
| 5         | S.T.(1")               | 32.3     | 83.6      | 31.5       | 29.0     | 24.0              |
| 5         | A-C( $\frac{1}{4}$ ")  | —        | —         | —          | —        | —                 |
| 5         | S.T.( $\frac{1}{4}$ ") | 37.9     | 94.4      | 38.0       | 36.5     | —                 |
| 6         | A-C(1")                | 48.2     | 72.6      | 1.5        | 2.5      | 2.0               |
| 6         | S.T.(1")               | 42.7     | 69.1      | 2.5        | 3.0      | 3.5               |
| 6         | A-C( $\frac{1}{4}$ ")  | 54.2     | 89.4      | 2.0        | 4.5      | —                 |

TABLE II-continued

| Alloy No.   | Condition (X-Sect.) | YS (ksi) | UTS (ksi) | Elong. (%) | R.A. (%) | Impact (ft.-lbs.) |
|-------------|---------------------|----------|-----------|------------|----------|-------------------|
| 6           | S.T.(1/4")          | 45.0     | 94.1      | 18.0       | 24.0     | —                 |
| 7           | A-C(1")             | 35.4     | 77.9      | 17.0       | 17.0     | 7.1               |
| 7           | S.T.(1")            | 32.7     | 80.2      | 27.0       | 25.5     | 14.0              |
| 7           | A-C(1/4")           | 39.0     | 83.3      | 14.5       | 17.5     | —                 |
| 7           | S.T.(1/4")          | 36.4     | 88.7      | 29.0       | 34.0     | —                 |
| 8           | A-C(1")             | 40.0     | 70.0      | 4.5        | 5.0      | 2.0               |
| 8           | S.T.(1")            | 36.6     | 70.2      | 7.5        | 6.0      | 7.0               |
| 8           | A-C(1/4")           | 50.3     | 88.4      | 7.5        | 4.5      | —                 |
| 8           | S.T.(1/4")          | 39.3     | 85.3      | 14.5       | 26.0     | —                 |
| 9           | A-C(1")             | 41.2     | 80.4      | 14.0       | 14.5     | 6.0               |
| 9           | S.T.(1")            | 37.3     | 84.1      | 24.0       | 24.5     | 17.0              |
| 9           | A-C(1/4")           | 45.5     | 93.3      | 16.5       | 17.0     | —                 |
| 9           | S.T.(1/4")          | 39.6     | 96.4      | 34.5       | 33.0     | —                 |
| 10          | A-C(1")             | 38.0     | 70.6      | 7.0        | 7.0      | 6.0               |
| 10          | S.T.(1")            | 37.3     | 84.1      | 24.0       | 24.5     | 17.0              |
| 10          | A-C(1/4")           | 46.1     | 84.1      | 7.5        | 4.5      | —                 |
| 10          | S.T.(1/4")          | 40.9     | 90.7      | 25.5       | 33.0     | —                 |
| 11          | A-C(1")             | 37.6     | 78.7      | 16.0       | 16.5     | 14.0              |
| 11          | S.T.(1")            | 36.5     | 79.8      | 22.5       | 21.0     | 17.0              |
| 11          | A-C(1/4")           | 41.6     | 89.6      | 18.0       | 17.5     | —                 |
| 11          | S.T.(1/4")          | 39.2     | 91.2      | 31.0       | 27.5     | —                 |
| 12          | A-C(1")             | 45.0     | 74.9      | 5.0        | 6.0      | 3.0               |
| 12          | S.T.(1")            | 40.1     | 76.6      | 10.0       | 11.0     | 6.0               |
| 12          | A-C(1/4")           | 52.9     | 94.9      | 9.0        | 6.0      | —                 |
| 12          | S.T.(1/4")          | 44.1     | 98.1      | 25.5       | 13.5     | —                 |
| 13          | A-C(1")             | 37.8     | 77.2      | 13.5       | 12.0     | 7.5               |
| 13          | S.T.(1")            | 35.4     | 80.2      | 19.0       | 12.5     | 11.0              |
| 14          | S.T.(1")            | 31.5     | 66.5      | 8.0        | 10.0     | —                 |
| 15          | S.T.(1")            | 32.3     | 68.3      | 9.5        | 11.0     | —                 |
| 16          | S.T.(1")            | 32.9     | 74.4      | 10.5       | 10.0     | —                 |
| 17          | S.T.(1")            | 32.2     | 71.7      | 14.5       | 12.0     | —                 |
| 18          | S.T.(1")            | 36.6     | 72.9      | 10.0       | 10.5     | —                 |
| 19          | S.T.(1")            | 42.1     | 75.7      | 5.0        | 5.5      | —                 |
| 20          | A-C(1")             | 37.8     | 74.1      | 11.5       | 13.0     | —                 |
| 20          | S.T.(1")            | 36.1     | 74.8      | 14.0       | 14.5     | —                 |
| Hardness Rc |                     |          |           |            |          |                   |
| 21          | A-C(1")             | ND       | 68.4      | 1.0        | 2.0      | 21                |
| 21          | S.T.(1")            | ND       | 66.2      | 1.0        | 1.5      | 19                |
| 22          | A.C.(1")            | ND       | 66.4      | 1.0        | 1.0      | 20                |
| 22          | S.T.(1")            | ND       | 63.0      | 1.5        | 1.0      | 17                |
| 23          | A.C.(1/4")          | 50.9     | 67.9      | 2.0        | 2.0      | 20                |
| 23          | S.T.(1/4")          | 53.1     | 73.1      | 1.5        | 2.0      | —                 |
| 24          | A.C.(1")            | ND       | 65.9      | 1.0        | 1.0      | 17                |
| 24          | S.T.(1")            | ND       | 68.0      | 2.0        | 2.0      | 16                |
| 25          | A.C.(1/4")          | 48.3     | 61.2      | 1.0        | 2.0      | 19                |
| 25          | S.T.(1/4")          | 48.7     | 70.3      | 2.0        | 2.0      | —                 |
| 26          | A.C.(1")            | ND       | 70.7      | 2.0        | 1.0      | 20                |
| 26          | S.T.(1")            | ND       | 69.5      | 3.0        | 1.0      | 19                |
| 27          | A.C.(1/4")          | 53.0     | 69.6      | 1.5        | 2.0      | —                 |
| 27          | S.T.(1/4")          | 48.2     | 71.8      | 1.5        | 2.0      | —                 |
| 28          | A.C.(1")            | 36.1     | 73.8      | 11.5       | 10.5     | —                 |
| 28          | S.T.(1")            | 36.4     | 74.0      | 11.0       | 12.5     | —                 |
| 28          | A.C.(1/4")          | 38.9     | 79.2      | 11.0       | 8.5      | —                 |
| 28          | S.T.(1/4")          | 32.7     | 82.3      | 16.5       | 6.0      | —                 |
| 29          | A.C.(1")            | 32.5     | 71.3      | 15.0       | 11.5     | —                 |
| 29          | S.T.(1")            | 31.6     | 74.0      | 19.0       | 16.5     | —                 |
| 29          | A.C.(1/4")          | 36.2     | 76.2      | 23.5       | 15.5     | —                 |
| 29          | S.T.(1/4")          | 34.3     | 88.1      | 45.5       | 27.0     | —                 |
| 30          | A.C.(1")            | 37.3     | 74.3      | 12.0       | 14.0     | —                 |
| 30          | S.T.(1")            | 37.1     | 75.2      | 10.5       | 14.5     | —                 |
| 30          | A.C.(1/4")          | 41.0     | 83.2      | 14.5       | 7.0      | —                 |
| 30          | S.T.(1/4")          | 43.8     | 82.2      | 14.5       | 10.0     | —                 |
| 31          | A.C.(1")            | 36.2     | 72.2      | 14.0       | 13.5     | —                 |
| 31          | S.T.(1")            | 37.7     | 75.3      | 17.0       | 19.5     | —                 |
| 31          | A.C.(1/4")          | 40.3     | 74.5      | 14.5       | 6.0      | —                 |
| 31          | S.T.(1/4")          | 37.8     | 83.3      | 25.5       | 19.5     | —                 |

YS = Yield Strength at 0.2% offset (Kips per square inch)

UTS = Ultimate Tensile Strength

Elong. = Tensile Elongation

R.A. = Reduction in Area

Impact = Impact Energy, Charpy V-Notch specimen (foot-pounds)

A-C(X-Sect.) = As-Cast(Cross-Section Thickness)

S.T. (X-Sect.) = Solution Treated one hour 2000°F, air cooled

Hardness(Rc) = Rockwell C hardness, average of two readings

N.D. = Not determined

It may be noted that all of the examples referred to in Tables I and II are characterized by yield strengths of at least 30,000 pounds per square inch (psi) at room temperature and that results obtained with specimens from 1/4-inch keel blocks of the steels with 0.3% to 0.7% boron illustrate a characteristic of at least 5% elongation in the rapidly solidified and solution-treated condition obtained by sand-casting in a 1/4-inch thick section

and solution treating one hour at 2,000°F. Moreover, it is notable that Table II illustrates that the solution treatment of compositions containing 0.3% to 0.7% boron in accordance with the invention resulted in improved ductility characteristics, particularly elongation and impact resistance, without detrimentally decreasing the ultimate tensile strength, and often somewhat increasing the tensile strength along with the improve-

ment in ductility.

The castings of invention had highly satisfactory smooth surfaces with good filling at corners in thin sections of the mold cavity and without any indications of metal-mold reactions, liquid-metal penetration of the mold, "burn on" or other types of surface roughness or defects of kinds resulting from excessively hot metal contact with molds. Moreover, CP-pattern castings of steels of the invention showed good freedom from folds, cold shuts or other defects such as occur if metal is poured too cold or lacks good fluidity. This CP (Chinese Puzzle) pattern, which is designed to test castability characteristics such as the ability of a molten metal to run through the passages of a complex mold with abrupt changes in flow direction that are conducive to turbulence, comprises a number of partially adjoining rectangular cavities of about three-sixteenths inch thickness. The CP pattern demands more of a melt than simply capability to remain fluid over the course of a long run, such as in a fluidity spiral, but requires many sharp changes in flow direction with the flow meeting and merging with itself, filling of many corners and flow through and filling of large thin flat surfaces, e.g., 1½ inches square by three-sixteenths inch thick.

In contrast with steels of the invention, e.g., alloys 4 through 12, and alloys 21 through 27 and 28 through 31, comparison tests wherein stainless steels of the Alloy Casting Institute Type CF-8 containing 0.05% carbon, 1.41% silicon, 1% manganese, 9.1% nickel, 18.4% chromium and 0.06% aluminum and another containing 0.10% carbon, 1.26% silicon, 1.3% manganese, 9.1% nickel, 19.2% chromium and 0.045% aluminum (without copper or boron) were cast at 2,950°F. in green sand molds of the same CP pattern showed inferior castability results with many cold shuts or fold defects in the castings. In comparison with the results of casting the CF-8 steel, the steels of the invention exhibited much better castability, particularly with success in avoiding entrapped films, folds and cold shuts when cast at 2,650°F. (alloys 4-12 and 28 through 31), or at 2,350°F. (alloys 23, 25 and 27) than did the results obtained casting CF-8 steel at 2,950°F.

Visual examination of flow-and-knit castings in the sand blasted condition showed that surface areas of flat sections near the sprues of the CF-8 castings were rougher than the corresponding surfaces on the castings of the steel of the invention. This reflects that the good castability of the steel of the invention enabled obtaining desirably smooth surfaces, with freedom from detrimental burn on and/or mold penetration, by pouring at desirably low temperatures while avoiding the undesirable kind of surface roughness that resulted from the need for pouring the CF-8 steel at the higher temperature (2,950°F.). The excessive surface roughness associated with the high pouring temperature of the CF-8 steel is particularly objectionable for commercial production since the rough surface with entrapped abrasive mold material introduces machining difficulties and considerably shortens the life of tool bits.

Resistance to hot tearing was evaluated with castings of the steels made in dry sand molds from a pattern having three cylindrical rods(arms) of different lengths, namely, 6 inches, 9 inches and 12 inches, each about one-half inch in diameter with flanges at each end which restrained the rods from shrinking during cooling. The general configuration of each of the three arms was similar to the flanged arm of the test pattern

illustrated in the paper by R. A. Rosenberg, M. C. Flemings and H. F. Taylor in Transactions of the American Foundrymen's Society, Vol. 68, 1960, pages 518-528, at page 519. Both the steels of the invention and the CF-8 steel resisted hot tearing on the 6-inch and 9-inch arms but did show hot-tearing on the 12-inch arm and thus the hot-tearing resistance of the steels of the invention (alloys 2 and 13) was deemed generally about as good as that of the CF-8 steel, which is usually considered to have at least moderately good resistance to hot tearing.

Good castability characteristics of the steel of the invention were also confirmed with fluidity spiral castings in dry sand molds and straight-run fluidity castings in iron molds. Steel castings of the invention which were cast at 2,650°F. in uncoated iron molds stripped cleanly from the molds with no difficulty and showed no tendency to burn-on, bond or detrimentally adhere to the mold.

Highly satisfactory, clean remelt characteristics which are needed for recycling of metal such as gates, risers and scrap castings were demonstrated with a series of ten recycle melts, or remelts, starting with metal from alloy 13. For each of the ten remelts in this recycle series, about two-thirds of the furnace charge was castings from the previous melt in the series and about one third of the charge was virgin raw material. Each remelt was deoxidized with 0.1% aluminum and 0.02% selenium was added. Each of the remelts was cast into a mold for hot-tear specimens; also, 1-inch thick keel blocks were poured from the first, fifth and tenth remelts to provide stock for tensile test specimens. Resistance to hot tearing remained uniformly good with satisfactory solidification and cooling in the six-inch and nine-inch arms but with some tearing on the 12-inch arms. Cleanliness of the remelts was consistently excellent. The remelts did not tend to generate or accumulate dross, oxide films or scum. Ranges of the chemical analyses reported from the ten remelts were: 0.051% to 0.096% carbon, 7.9% to 8.6 % nickel, 15.2% to 17.1% chromium, 2.80% to 3.15% silicon, 16.4% to 17.9% manganese, 0.37% to 0.51% boron and 1.93% to 2.14% copper. Tensile strength and ductility characteristics of the remelts were consistently satisfactory, with room temperature tensile and impact characteristics of 37.7 to 40.4 ksi YS, 73.8 to 77.2 ksi UTS, 7 to 13.5% Elong. and 4.5 to 7.5 ft.-lb. Impact, in the As-Cast condition; and 34.8 to 37.1 ksi YS, 80.2 to 80.6 ksi UTS, 15 to 19% Elong. and 9 to 13 ft.-lb. Impact in the Solution Treated Condition.

Alloys 22, 24 and 26 were remelted in gas-fired furnaces and cast at 2,350°F. into CP-pattern green sand molds. Visual examination of the resulting castings showed that these remelted alloys successfully filled mold cavities about three-sixteenths inch thick by 1½ inches square and produced satisfactory castings with good smooth surfaces and sharp definition without entrapped films, folds or cold shuts when poured at 2,350°F., thus confirming excellent castability.

In other instances of demonstrating good remelt castability characteristics, steels of the invention, e.g., embodiments of an advantageous composition containing about 8% to 10% nickel, 15% or 17.5% to 19.5% chromium, 0.02% to 0.1% carbon, 2.75% to 3.25% or 3.5% silicon, 16% to 18% or 19% manganese, 0.45% to 0.7% boron, 1.5% to 2.5% copper and balance essentially iron, were remelted and die cast (under pressure) at about 2,450°F. to 2,600°F. The resulting stainless steel

die castings of the invention stripped cleanly from the metal molds, were well-filled and had highly satisfactory smooth, sharply defined surfaces.

Stainless steels of the invention, e.g., alloy 8 in the as-cast condition and in the solution treated condition, exhibited good machinability when drilled with high speed steel drills.

A specimen of alloy 7 had a hardness of 51 Rockwell A in the solution annealed condition and had the same hardness of 51 Rockwell A after aging at 1,250°F. for 15 hours following the solution treatment.

Brazing is recommended if there is need to join the steel to itself. Specimens of a steel of the invention containing about 0.082% carbon, 8.4% nickel, 15.9% chromium, 3.18% silicon, 17.5% manganese, 2.11% copper and 0.48% boron were satisfactorily brazed together by torch brazing using a commercial silver-solder brazing alloy. Subsequent testing showed that the resultant brazed join had good impact resistance; moreover, metallurgical examination showed that the brazing alloy flowed satisfactorily with good wetting of the steel, and the brazed steel surfaces were free from intergranular penetration.

Cast steels of the invention, advantageously in the solution treated condition, and with boron in the range of 0.3% to 0.7%, have good corrosion resistance that is clearly superior to the corrosion resistance of martensitic stainless steels, e.g., ACI Types CA-15 and CB-30, and approaches or approximates, and in some instances equals, the corrosion resistance of austenitic stainless steels, e.g., Type CF-8, in many respects. Results of CASS (Copper Accelerated Salt Spray) tests corresponding to ASTM B368-61T confirmed that steels of the invention have satisfactory resistance to pitting in salt spray. For instance, solution treated specimens of alloys 14 through 19 (containing about 10% to 26% nickel) which were subjected to CASS tests of seven days duration exhibited good resistance to pitting and to general corrosion in salt spray that was about as good as that of Type CF-8 steel, with the best corrosion resistance being evidenced by alloys 14, 15 and 16. In CASS tests of 24 hours duration, specimens of alloys 4 through 12 in the solution treated condition successfully resisted pitting and showed general corrosion resistance between that of Types CB-30 and CF-8. Corrosion tests of steels 4 through 7 in deaerated 5%  $H_2SO_4$  at room temperature showed corrosion resistance intermediate between that of Types CB-30 and CF-8.

The present invention is particularly applicable to economical production of cast-to-shape stainless steel articles including home and industrial housing hardware, e.g., door handles and door stops, plumbing hardware, e.g., pipe fittings, faucets and valve bodies, marine hardware, e.g., rope cleats, and also including decorative trim, escutcheon plates, pump housings and trivets. The invention is applicable to providing many kinds of articles that are commonly made of cast brass and in this regard the corrosion resistant characteristics of the subject steels are deemed especially beneficial for resisting corrosive attack by ammonia, including moist ammonia and ammoniacal cleansers, such as has been found detrimental to brass. While utility referred to hereinbefore is largely at room temperature, it should be understood the present steels have useful strength at temperatures substantially below and above room temperature, such as from sub-zero temperatures up to about 1,000°F. or higher.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

I claim:

1. An austenitic nickel-chromium stainless steel consisting essentially of 6% to about 28% nickel, about 14% to about 25% chromium, 2% to about 5% silicon, 0.3% to about 0.7% boron, up to about 0.15% carbon, up to about 20% manganese, up to about 3% copper, up to about 8% molybdenum, up to about 1% columbium and balance iron and wherein the amounts of nickel, chromium, silicon, and boron and any manganese and molybdenum in the alloy are correlated in accordance with the relationship

$$8(\%Ni+\%Mn)-1.5(\%Cr+\%Mo)+22(\%Si+284(\%B)) \text{ equal at least } 360;$$

said steel being characterized by castability superior to that of austenitic steels of the A.C.I. CF-8 type, as determined by relative freedom from cold shut defects when cast in three-sixteenths-inch thick by 1½-inch interlocking squares in green sand molds according to the Chinese Puzzle pattern, and additionally characterized by corrosion resistance superior to that of martensitic-ferritic steels of the A.C.I. CA-15 and CB-30 types, as determined by resistance to pitting and general corrosion in salt-spray CASS tests corresponding to ASTM B368-61T.

2. An austenitic nickel-chromium stainless steel consisting essentially of 8% to 10% nickel, 17.5% to 19.5% chromium, 0.02% to 0.1% carbon, 2.75% to 3.25% silicon, 0.45% to 0.7% boron, 16% to 18% manganese, 1.5% to 2.5% copper up to about 8% molybdenum, up to 1% columbium, and balance essentially iron and wherein the composition is controlled in accordance with the relationship

$$8(\%Ni+\%Mn)-1.5(\%Cr+\%Mo)+22(\%Si)+284(\%B) \text{ equal at least } 385.$$

3. An austenitic nickel-chromium stainless steel consisting essentially of 23.5% to 26% nickel, 18% to 20% chromium, 0.02% to 0.08% carbon, 3% to 3.5% silicon, 0.55% to 0.7% boron, 1% to 2% manganese, 2.2% to 2.7% copper 2.3% to 6.5% molybdenum and balance essentially iron and wherein the composition is controlled in accordance with the relationship

$$8(\%Ni+\%Mn)-1.5(\%Cr+\%Mo)+22(\%Si+284(\%B)) \text{ equal at least } 360.$$

4. An austenitic nickel-chromium stainless steel casting characterized by (a) a room temperature tensile elongation of at least about 5%, (b) a room temperature yield strength of at least 25,000 pounds per square inch, (c) a stable austenitic cast microstructure containing austenitic dendrites and (d) being formed from a steel characterized at 2,650°F. by a molten condition possessing good castability for flowing and knitting and resisting formation of cold shut defects and for merging and solidifying in the form of continuously sound cast metal in thin, relatively large area, green-sand mold cavities of three-sixteenths-inch thickness by 1½ inch square area interlocked in patterns conducive to turbu-

lent flow of molten metal, said steel consisting essentially of 8% to about 30% nickel, about 14% to about 26% chromium, 2% to 3.8% silicon, 0.2% to about 0.7% boron, up to about 0.15% carbon, up to about 20% manganese, up to about 3% copper, up to about 6% molybdenum, up to about 1% columbium, up to about 0.2% phosphorus and balance iron and wherein the amounts of nickel, chromium, silicon, boron and any manganese, molybdenum and phosphorus in the alloy are correlated in accordance with the relationship

$$8\% \\ (\%Ni+Mn)-1.5(\%Cr+\%Mo)+22(- \\ \%Si)+284(\%B)+189(\%P) \text{ equal at least } 180.$$

5. A process comprising establishing a molten bath of the steel set forth in claim 4, pouring the molten steel into a mold and then solidifying the steel to thereby produce a cast-to-shape stainless steel article.

6. A stainless steel casting as set forth in claim 4 wherein the amount of any manganese present does not exceed 5%.

7. An austenitic nickel-chromium stainless steel consisting essentially of casting according to claim 4 about 8% to 14% nickel, 16% to 20% chromium, 2.5% to 3.5% silicon, 0.25% to 0.55% boron, 0.2% to 2.5% manganese, up to 4% molybdenum and up to 2% copper.

8. An austenitic nickel-chromium stainless steel consisting essentially of 6% to about 30% nickel, about 14% to about 26% chromium, 2% to about 5% silicon, 0.2% to 1.4% boron, up to about 0.15% carbon, up to about 20% manganese, up to about 3% copper, up to about 8% molybdenum, up to 1.4% phosphorus, up to about 1% columbium and balance iron and wherein the amounts of nickel, chromium, silicon, boron and any manganese, molybdenum and phosphorus in the alloy are correlated in accordance with the relationship

5

10

15

20

25

30

35

40

8\%(%Ni+Mn)-1.5(%Cr+\%Mo)+22(- \\ \%Si)+284(\%B)+189(\%P) \text{ equal at least } 180;

said steel being characterized in the molten condition by castability superior to that of austenitic steels of the A.C.I. CF-8 type, as determined by relative freedom from cold shut defects when cast in three-sixteenths-inch thick by 1½-inch interlocking squares in green sand molds according to the Chinese Puzzle pattern, and in the solid condition by a non-age hardenable austenitic microstructure having corrosion resistance superior to that of martensitic-ferritic steels of the A.C.I. CA-15 and CB-30 types, as determined by resistance to pitting and general corrosion in salt-spray CASS tests corresponding to ASTM B368-61T.

9. A stainless steel as set forth in claim 8 containing at least 8% nickel.

10. A stainless steel as set forth in claim 8 containing 2.5% to 3.8% silicon.

11. A stainless steel as set forth in claim 8 containing 8% to 14% nickel, 16% to 20% chromium, 0.2% to 0.55% boron, 0.2% to 2.5% manganese, up to 4% molybdenum and up to 0.2% phosphorus.

12. A process comprising preparing a molten bath of steel having a composition in accordance with claim 8, casting the steel into a mold and solidifying the steel in the mold.

13. A process as set forth in claim 12 wherein the steel is solidified in an expendable refractory mold.

14. A process as set forth in claim 12 wherein the steel is solidified in a metal mold.

15. A process as set forth in claim 14 wherein the steel is die cast under pressure.

16. A process as set forth in claim 12 wherein the steel is rapidly solidified at a rate at least equivalent to solidification of a ¼-inch thick cross-section in a dry sand mold and is thereafter solution-treated for at least one-half hour at 1,850°F. to 2,050°F.

\* \* \* \* \*

45

50

55

60

65